

# UNITED STATES PATENT OFFICE.

WILLIAM D. SNOW, ALBERT B. LUECKE, AND DAVID L. SNOW, OF PHILADELPHIA, PENNSYLVANIA.

## LINOLEUM.

No. 911,341.

Specification of Letters Patent.

Patented Feb. 2, 1909.

Application filed March 14, 1908. Serial No. 421,144.

*To all whom it may concern:*

Be it known that we, WILLIAM D. SNOW, ALBERT B. LUECKE, and DAVID L. SNOW, citizens of the United States, and residents 5 of the city of Philadelphia, county of Philadelphia, and State of Pennsylvania, have jointly invented certain Improvements in Linoleum, of which the following is a specification.

10 This invention consists primarily of a combination of oxidized linseed oil and ground leather, with the addition usually of driers and coloring matter, which are thoroughly mixed and sheeted for use, as floor cloths, in 15 book binding, as carriage covers, in upholstery, and otherwise, as a cheap substitute for leather.

In practice we have produced a very satisfactory product by intimately mixing together the specified ingredients in the proportions of one pound of oxidized linseed oil, two pounds of ground leather, two ounces of litharge, and such coloring matter as may be desired, which, upon rolling into 25 sheets, both upon and without a woven backing fabric, gave a smooth, durable and inexpensive cloth suitable for the uses specified.

We may also use in combination with the reduced leather and linseed oil more or less 30 corn oil.

Having described our invention, we claim:

1. The combination of reduced leather and oxidized linseed oil substantially as specified. 35
2. The combination of reduced leather, oxidized linseed oil and a drier, substantially as specified.
3. The combination of ground leather and oxidized linseed oil substantially of the 40 proportions by weight of one part of oxidized oil to two parts of ground leather, substantially as specified.
4. The combination of intimately mixed ground leather and oxidized linseed oil with 45 a woven backing fabric, substantially as specified.
5. The combination of oxidized linseed oil, ground leather, litharge and coloring matter in approximately the proportions of one 50 pound of oil, two pounds of leather and two ounces of litharge.

In witness wherof we have hereunto set our names this 10th day of March, A. D. 1908, in the presence of the subscribing witnesses.

WILLIAM D. SNOW.  
ALBERT B. LUECKE.  
DAVID L. SNOW.

Witnesses:

JESSE G. MYERS,  
LYNDELL MYERS.